

# United States Patent [19]

Inaba et al.

[11] Patent Number: 4,634,629

[45] Date of Patent: Jan. 6, 1987

[54] LIFT-OFF TAPE USABLE MANY TIMES

[75] Inventors: **Masatsugu Inaba, Settsu; Takumi Murasaki, Neyagawa, both of Japan**

[73] Assignee: **Fuji Kagakushi Kogyo Co., Ltd., Japan**

[21] Appl. No.: **709,045**

[22] Filed: **Mar. 7, 1985**

[30] Foreign Application Priority Data

Mar. 9, 1984 [JP] Japan ..... 59-45950  
Nov. 27, 1984 [JP] Japan ..... 59-251176

[51] Int. Cl. <sup>4</sup> ..... **C09J 7/02; B32B 27/08;  
B41J 31/05**

[52] U.S. Cl. ..... **428/343; 400/696;  
428/355; 428/474.4; 428/914**

[58] Field of Search ..... **428/343, 355, 914, 474.4;  
400/696**

[56]

## References Cited

### U.S. PATENT DOCUMENTS

4,406,912 9/1983 Downing ..... 428/343 X  
4,434,207 2/1984 Franey ..... 428/343

Primary Examiner—Thomas J. Herbert  
Attorney, Agent, or Firm—Thomas L. Tully

[57]

## ABSTRACT

A lift-off tape capable of being used many times which comprises a foundation and an adhesive layer provided on one major surface of the foundation, said adhesive layer containing a plasticizer capable of plasticizing a polyamide resin which is a main component of the vehicle of a correctable ink. The lift-off tape can be used many times to remove erroneous typed impressions of a correctable ink which contains a polyamide resin as a main component of the vehicle thereof.

17 Claims, No Drawings

## LIFT-OFF TAPE USABLE MANY TIMES

## BACKGROUND OF THE INVENTION

The present invention relates to a lift-off tape. More particularly, it relates to a lift-off tape for peeling off or removing erroneous ink impressions formed by impact on recording paper from a correctable ink ribbon.

Heretofore, in impact typewriters, there have often been used adhesive correction tapes called "lift-off tape" which are normally tacky or made tacky by the application of pressure or other stress even though they are normally nontacky, and have the capability of peeling off ink impressions.

Such correction tape is so designed that erroneous typed ink impressions on recording paper are peeled off and transferred onto the tape by typing using usual typewriters. Such lift-off tapes are disclosed, e.g., in Japanese Published Unexamined Patent Application Nos. 41941/1979 and 122315/1975.

In the case of a conventional lift-off tape, its portions that are once used are covered with the correctable ink of the removed ink impression. When the used portions are reused, the correctable ink will reduce the peeling-off force of the adhesive layer to the extent that impressions cannot be removed as neatly as when the tape is used for the first time. Thus, it has been considered in prior technique that the lift-off tape is usable only once.

## SUMMARY OF THE INVENTION

It is an object of the invention to provide a lift-off tape which can be used many times even where its portions are covered with correctable ink.

This and other objects of the invention will become apparent from the description hereinafter.

The present invention provides a lift-off tape which can be used many times, comprising a foundation, and an adhesive layer provided on one major surface of the foundation, the adhesive layer containing a plasticizer capable of plasticizing a polyamide resin which is a main component of the vehicle of a correctable ink.

## DETAILED DESCRIPTION

The aforesaid features of the invention enable the correctable ink which has adhered to the adhesive layer (hereinafter referred to as lift-off layer) of the lift-off tape to develop the impression peeling-off action, thus enabling the tape to be used many times.

Stated in more detail, correctable ink on correctable ink ribbons is generally in the form of a weak or frail film containing a polyamide resin as a main component of the vehicle for retaining the capability of the lift-off tape to peel off impressions from recording paper. When impressions of such correctable ink adhere to the above-specified lift-off layer, the ink is rendered tacky by the action of the plasticizer which has migrated into the ink, thus developing the ability to pick off typed impressions.

Such function and effect of the specific plasticizer contained in the lift-off layer make it possible to use a lift-off tape many times, which previously has been considered impossible.

The invention will now be described more concretely.

The lift-off layer in the lift-off tape of the invention is a layer formed by incorporating the above-specified

plasticizer in a usual lift-off layer composed mainly of a rubber-like resin and a tackifier.

The rubber-like resin is a binder for fixing the tackifier and other components to the foundation.

5 The plasticizer used in the invention may be any plasticizer that exerts a plasticizing action on the polyamide resin in the correctable ink. Typical examples of plasticizers of such a nature are oleic acid, isostearic acid, polyoxyethylene castor oil, polyoxyethylene oleylamine, coconut oil fatty acid diethanolamide, polyoxyethylene lauryl ether, polyoxyethylene nonylphenyl ether, di(polyoxyethylene alkyl ether) phosphate, trimethylolpropane monoerucate, sorbitan monolaurate, sorbitan sesquioleate, and polyoxyethylene sorbitol tetraoleate. These plasticizers may be used singly or as mixtures of two or more of them.

In a combination of the plasticizer with a tackifier which is a main component of the lift-off layer, the plasticizer may have or may not have a plasticizing action on the tackifier.

In the case of using a plasticizer which has substantially no plasticizing action on the tackifier, the lift-off layer itself does not become plasticized and there is no possibility that the lift-off layer will become extremely softened to the extent of being peeled off from the foundation, or that the softness of the lift-off layer will be influenced very much by a decrease of the content of the plasticizer in the lift-off layer which is caused by repeated uses of the lift-off tape. Thus, there will take place no change which causes interference with usage, such as hardening of the layer. However, when a plasticizer having a plasticizer action on the tackifier is used, it is not always necessary to use separately an agent which assists the plasticization of the lift-off layer.

35 The amount of the plasticizer used is preferably in the range of 0.1 to 50 parts (parts by weight, hereinafter the same) when the amount of the tackifier used is taken to be 10 parts. Particularly in the case of a plasticizer having no plasticizing action on the tackifier, the amount is 40 preferably in the range of 0.5 to 30 parts, more preferably 2 to 20 parts per 10 parts of the tackifier. Further, in the case of a plasticizer having a plasticizing action on the tackifier, the amount is preferably in the range of 0.5 to 20 parts, more preferably 2 to 10 parts per 10 parts of the tackifier. If the amount of the plasticizer used is less than the above range, the plasticization of the correctable ink peeled off from the recording paper and adhering to the lift-off layer would be insufficient, considerably degrading the removal of impressions in reuse. On the other hand, if it is more than the above range, the correctable ink peeled off from the recording paper and adhering to the lift-off layer would be plasticized too much, involving the danger that the correctable ink plasticized would be transferred again to the recording paper during reuse.

45 Usually, the plasticizer is present in the lift-off layer in such a state that it is homogeneously dissolved or dispersed in other components. In particular, in the case 50 of a plasticizer having no plasticizing action on the tackifier, it may be present in the lift-off layer in such a state that it is contained in microcapsules, the strength of which is adjusted so that the microcapsules can be collapsed by the application of type pressure.

60 Examples of the rubber-like resin include, for instance, styrene-butadiene copolymer, polyester resin, vinyl chloride-vinyl acetate copolymer, polyvinyl butyral, and ethylene-vinyl acetate copolymer.



TABLE 1-continued

| Component                         | Ex. 1 | Ex. 2 | Ex. 3 | Ex. 4 | Ex. 5 | Ex. 6 | Ex. 7 |
|-----------------------------------|-------|-------|-------|-------|-------|-------|-------|
| Paraffin wax                      | —     | —     | —     | —     | —     | 2     | —     |
| Low molecular weight polyethylene | —     | —     | —     | —     | —     | —     | 1     |
| <u>Lubricant</u>                  |       |       |       |       |       |       |       |
| Zinc molybdate                    | —     | —     | —     | —     | 1     | —     | —     |
| Talc                              | —     | —     | —     | —     | —     | —     | 1     |
| <u>Volatile solvent</u>           |       |       |       |       |       |       |       |
| Toluene                           | 40    | 60    | 60    | 60    | 60    | 40    | 60    |
| Isopropyl alcohol                 | 20    | —     | —     | —     | —     | 20    | —     |

Note:

The unit of numerical values in Table 1 is parts.

## COMPARATIVE EXAMPLES 1 TO 7

Seven kinds of lift-off tapes were prepared in the same manner as in Examples 1 to 7 except that the plasticizer for polyamide was removed from each composition shown in Table 1. These lift-off tapes were tested for their ability of removing impressions, in the same manner as in the aforesaid test. As a result, it was found that at the clearness of retyped impressions after the 3rd or 4th time of use was considerably inferior to that

15 spect to the lift-off tapes, the ability of peeling-off or removing impressions was determined in the same manner as in Examples 1 to 7.

20 Removal operation was repeated throughout the length of the lift-off tape, and it was found that the same quality of removal as for the 1st time of use was exhibited until about the 4th time of use. When the tape was used more than four times, fine ink dust was left on the recording paper, but this little influenced the clearness of retyped impressions.

TABLE 2

| Component                                    | Ex. 8 | Ex. 9 | Ex. 10 | Ex. 11 | Ex. 12 |
|----------------------------------------------|-------|-------|--------|--------|--------|
| <u>Rubber-like resin</u>                     |       |       |        |        |        |
| Styrene-butadiene copolymer                  | 10    | —     | —      | 6      | —      |
| Polyvinyl butyral                            | —     | 10    | —      | —      | —      |
| Ethylene-vinyl acetate copolymer             | —     | —     | 10     | —      | 10     |
| <u>Tackifier</u>                             |       |       |        |        |        |
| Styrene resin                                | 8     | —     | —      | —      | —      |
| Acrylic resin                                | —     | 8     | —      | 10     | —      |
| $\alpha$ -Pinene resin                       | —     | —     | 10     | —      | 10     |
| <u>Non-volatile liquid</u>                   |       |       |        |        |        |
| Terpene oligomer                             | —     | 1     | —      | —      | —      |
| Liquid type polybutadiene                    | —     | —     | —      | 2      | —      |
| Liquid type polybutene                       | —     | —     | —      | —      | 2      |
| <u>Plasticizer for polyamide</u>             |       |       |        |        |        |
| Trimethylolpropane monoerucate               | 7     | —     | —      | —      | —      |
| Polyoxyethylene oleylamide                   | —     | —     | 5      | —      | —      |
| Sorbitan monolaurate                         | —     | —     | —      | 2      | —      |
| Oleic acid                                   | —     | 5     | —      | —      | 2      |
| Isostearic acid                              | —     | —     | —      | —      | 1      |
| <u>Tackiness-reducing agent or Lubricant</u> |       |       |        |        |        |
| Low molecular weight polyethylene            | —     | —     | —      | —      | 5      |
| Finely powdered silica                       | —     | —     | 2      | —      | —      |
| Zinc molybdate                               | —     | —     | 3      | 10     | —      |
| Talc                                         | —     | —     | —      | —      | 5      |
| <u>Volatile solvent</u>                      |       |       |        |        |        |
| Toluene                                      | 70    | 50    | 70     | 70     | 65     |
| Isopropyl alcohol                            | —     | 25    | —      | —      | —      |

Note:

The unit of numerical values in Table 2 is parts.

obtained after the 4th time of use in each of Examples 1 to 7.

In addition, in the case where the amount of plasticizer used in each of Examples 1 to 7 was reduced to 0.1 55 part per 10 parts of the tackifier, it was after the tape was repeatedly used more than about 6 times that the unclarity of retyped impressions was the same as when the tape in each Comparative Example was used for the 3rd time.

## EXAMPLES 8 TO 12

In these Examples, a combination of a tackifier and a plasticizer having a plasticizing action thereon was used.

The same procedures as in Examples 1 to 7 except that each of lift-off layer compositions shown in Table 2 was used were repeated to give lift-off tapes. With re-

## COMPARATIVE EXAMPLES 8 TO 12

Five kinds of lift-off tapes were prepared in the same manner as in Examples 8 to 12 except that polybutadiene was used as a plasticizer which hardly or does not at all plasticize polyamide resin instead of the plasticizers shown in Table 2. These tapes were tested for their ability of removing impressions in the same manner as in Example 1 to 7. As a result, it was found that the clearness of retyped impressions after second time of use was considerably inferior to that obtained after the 4th time of use in each of Examples 8 to 12.

As is clear from these results, the lift-off tape of the present invention can be used many times, which fact has heretofore been considered impossible.

In addition to the ingredients or elements used in the Examples, other ingredients or elements can be used in the Examples as set forth in the specification to obtain substantially the same results.

What we claim is:

1. A reusable pressure-sensitive lift-off correction element for removing correctable images of type ink containing a polyamide resin which are typed onto an original sheet, which comprises a flexible foundation, and a pressure-sensitive layer coated on one surface of the flexible foundation, said pressure-sensitive layer comprising a rubber-like resin binder material, a tackifier resin, and from 0.5 to 50 parts by weight, per each 10 parts by weight of the tackifier resin of a plasticizer for plasticizing the polyamide resin of the correctable images of type ink, whereby correctable images which are adhered to said layer and removed from said original sheet are rendered adhesive by said plasticizing action to permit additional correctable images of type ink to be adhered thereto during reuse.

2. The reusable pressure-sensitive lift-off correction element of claim 1, wherein said rubber-like resin binder material is selected from the group consisting of styrene-butadiene copolymer, polyester resin, vinyl chloride-vinyl acetate copolymer, polyvinyl butyral and ethylene-vinyl acetate copolymer.

3. The reusable pressure-sensitive lift-off correction element of claim 2, wherein said tackifier resin is selected from the group consisting of epoxy resin, styrene resin, acrylic resin, ketone resin, xylene resin, gum rosin and alpha pinene resin.

4. A reusable pressure-sensitive lift-off correction element for removing correctable images of type ink containing a polyamide resin which are typed onto an original sheet, which comprises a flexible foundation, and a pressure-sensitive layer coated on one surface of the flexible foundation, said pressure-sensitive layer comprising a rubber-like resin binder material selected from the group consisting of styrene-butadiene copolymer, polyester resin, vinyl chloride-vinyl acetate copolymer, polyvinyl butyral and ethylene-vinyl acetate copolymer, a tackifier resin, and from 0.5 to 50 parts by weight, per each 10 parts by weight of the tackifier resin of a plasticizer for plasticizing the polyamide resin of the correctable images of type ink, whereby correctable images which are adhered to said layer and removed from said original sheet are rendered adhesive by said plasticizing action to permit additional correctable images of type ink to be adhered thereto during reuse.

5. A reusable pressure-sensitive lift-off correction element having a pressure-adhesive layer, each area of which is capable of bonding to and lifting-off a plurality of correctable images which are typed onto an original sheet with correctable imaging composition containing a polyamide resin binder material, said element comprising a flexible foundation having a pressure-adhesive layer on one surface thereof, said layer comprising 0.5

to 100 parts by weight of a rubber-like resin binder material selected from the group consisting of styrene-butadiene copolymer, polyester, vinyl chloride-vinyl acetate, polyvinyl butyral and ethylene-vinyl acetate,

5 10 parts by weight of a tackifier resin selected from the group consisting of epoxy, styrene, acrylic, ketone, xylene, gum rosin, and alpha pinene resins, and 0.5 to 50 parts by weight of a plasticizer which has a plasticizing action on the polyamide resin of the correctable images, whereby correctable images which are adhered to said layer and removed from said original sheet are rendered adhesive by said plasticizing action to permit additional correctable images to be adhered thereto during reuse.

6. The reusable pressure-sensitive lift-off correction element of claim 5, wherein said plasticizer is oleic acid.

7. The reusable pressure-sensitive lift-off correction element of claim 5, wherein said plasticizer is polyoxyethylene oleylamide.

8. The reusable pressure-sensitive lift-off correction element of claim 5, wherein said plasticizer is coconut oil fatty acid diethanolamide.

9. The reusable pressure-sensitive lift-off correction element of claim 5, wherein said plasticizer is polyoxyethylene sorbitol tetraoleate.

10. The reusable pressure-sensitive lift-off correction element of claim 5, wherein said plasticizer is polyoxyethylene nonylphenyl ether.

11. The reusable pressure-sensitive lift-off correction element of claim 5, wherein said plasticizer is trimethylolpropane monoerucate.

12. The reusable pressure-sensitive lift-off correction element of claim 5, wherein said plasticizer is sorbitan monolaurate.

13. An element according to claim 5 in which the pressure-adhesive layer also contains up to 30 parts by weight of a tackiness-reducing agent.

14. An element according to claim 5 in which the pressure-adhesive layer comprises 10 parts by weight of the tackifier resin, 0.5 to 20 parts by weight of the plasticizer for the polyamide resin which also has a plasticizing effect on the tackifier resin, and 1 to 30 parts by weight of the rubber-like resin.

15. An element according to claim 14 in which the pressure-adhesive layer comprises 10 parts by weight of the tackifier resin, 2 to 10 parts by weight of the plasticizer for the polyamide resin and 5 to 20 parts by weight of rubber-like resin.

16. An element according to claim 5 in which the plasticizer for the polyamide resin has no plasticizing action on the tackifier resin, and the pressure-adhesive layer also contains a nonvolatile liquid which does plasticize the tackifier resin.

17. An element according to claim 16 containing 10 parts by weight of the tackifier resin, 0.5 to 30 parts by weight of the plasticizer for the polyamide resin and 1 to 30 parts by weight of the nonvolatile liquid.

\* \* \* \* \*